

# UNITED STATES PATENT OFFICE.

SEIKO SHIGETA, OF TOKYO, JAPAN.

## MOLYBDENUM BRONZE.

1,319,537.

Specification of Letters Patent.

Patented Oct. 21, 1919.

No Drawing.

Application filed June 3, 1918. Serial No. 237,940.

To all whom it may concern:

Be it known that I, SEIKO SHIGETA, a subject of the Empire of Japan, residing at No. 23 Minamifutabacho, Honjo-Ku, Tokyo, 5 Japan, have invented certain new and useful improvements in Molybdenum Bronze, of which the following is a specification.

My invention relates to a molybdenum bronze consisting of an alloy of copper, 10 aluminium, molybdenum and tungsten.

The object of my invention is the production of a new practical alloy which has properties similar to gold as to color, brilliancy, immutability and ductility, etc.

The ingredients of my alloy are copper, aluminium, tungsten and molybdenum, and this alloy is to be produced, for an example, as follows: Copper, molybdenum and tungsten, each in due proportion, are mixed together in a suitable crucible, and after they have been heated and melted, aluminium is to be added thereto step by step in small quantities at a time, until the necessary proportion is present, and the whole mixture 25 is melted uniformly.

In preparing the alloy I prefer to use the said ingredients in the following proportions:

|    |                  |     |
|----|------------------|-----|
| 39 | Copper -----     | 80% |
|    | Aluminium -----  | 10% |
|    | Molybdenum ----- | 5%  |
|    | Tungsten -----   | 5%  |

Among the above ingredients, molybdenum is used to bring the principal cause to afford the characteristic as to the color, brilliancy, immutability and ductility of the alloy, and tungsten acts mainly to increase

the acid-proof property and tensile strength of the same. If tungsten is used in excess, 40 however, this tends to decrease the ductility of the alloy and adds a tinge of red to the same, resulting in an inferior quality of alloy, therefore, it is necessary to suitably adjust the proportion of tungsten according 45 to the use of the alloy to be produced.

My alloy has a color similar to that of eighteen to twenty carat gold, its polished surface possesses a permanent brilliancy which does not become affected by air and 50 moisture, its ductility is high so that it can be drawn into a fine wire or can be worked into a thin leaf, it is not eroded by the action of acid or alkali, its tensile strength is great, it has an appropriate hardness so 55 as to suit it for hammering and engraving, and, as a whole, my alloy possesses all the desirable properties of a practical substitute of gold.

I claim:

1. A molybdenum bronze consisting of an alloy of a large amount of copper, a much smaller amount of aluminum, and still smaller, but substantial, amounts of molybdenum and tungsten, said alloy having the appearance and many of the other physical properties of gold. 60

2. An alloy containing about 80% copper, about 10% aluminum and about 5% each of molybdenum and tungsten. 65 70

In testimony whereof I affix my signature in presence of two witnesses.

SEIKO SHIGETA.

Witnesses:

DEN KIDO,  
EISHIRO ABE.